

July 25, 1950

C. C. MA

2,516,227

ELECTROPLATING OF CHROMIUM-MOLYBDENUM ALLOYS

Filed March 10, 1945



INVENTOR  
CHUK CHING MA

BY *J.W. Newhouse*  
ATTORNEY

## UNITED STATES PATENT OFFICE

2,516,227

## ELECTROPLATING OF CHROMIUM-MOLYBDENUM ALLOYS

Chuk Ching Ma, Orange, N. J., assignor to Westinghouse Electric Corporation, East Pittsburgh, Pa., a corporation of Pennsylvania

Application March 10, 1945, Serial No. 582,004

2 Claims. (Cl. 204—43)

1

This invention relates to electroplating and, more particularly, to such a process applied to alloys of chromium and molybdenum.

The principal object of my invention, generally considered, is to deposit alloys of chromium and molybdenum from aqueous solutions in dense closely-adherent form.

Another object of my invention is to plate alloys of chromium and molybdenum from aqueous solutions, such alloys to contain from 1% to 30% of molybdenum.

A further object of my invention is to coat base metal, such as copper and iron, with a dense, closely-adherent plating of an alloy such as chromium-molybdenum which is highly resistant to oxidation and the corrosive action of chemicals.

Other objects and advantages of the invention will become apparent as the description proceeds.

Referring to the drawing, the single figure shows in vertical section a container holding a plating bath, in which are immersed a pair of co-operating electrodes.

Chromium may be plated from solution, but is ordinarily formed by the reduction of chromium oxide by aluminum. Molybdenum in the metallic form is producible by reduction of the oxide by carbon or hydrogen. However, it cannot be deposited by itself from aqueous solution as a plating. Both chromium and molybdenum, however, are in group VI of the periodic table of the elements and there, therefore, appeared to be a possibility of co-deposition from an aqueous solution which contained both chromium and molybdenum ions.

For the purpose of determining whether this was possible, I dissolved molybdenum trioxide in a solution of chromic acid and was able to deposit alloys of chromium and molybdenum on a cathode immersed in said solution. I found that such plating was in dense closely-adherent form, thereby well serving to protect the metal on which deposited from oxidation and corrosive action.

The protection of readily oxidizable metals such as iron, copper, etc., by plating the same with a densely-adherent coating of an alloy of

chromium and molybdenum in accordance with my invention is feasible because of the unusual properties of the alloying metals. These properties supplement one another so that the alloy is resistant to more chemicals than either of the constituents thereof. For example, while chromium is soluble in hydrochloric and cold dilute hydrofluoric acids, molybdenum is insoluble, so that an alloy of the two is resistant to these acids. On the other hand, while molybdenum is soluble in nitric acid, chromium is insoluble so that the alloy is resistant to that acid. While chromium is soluble in dilute sulphuric acid, molybdenum is only slightly soluble so that the alloy is resistant to that acid.

Referring now to the drawing, there is shown a container 1 in which is a solution 2 of molybdate acid in chromic acid. The proportion is desirably about three times the weight of chromic oxide ( $\text{CrO}_3$ ) that there is of molybdenum trioxide ( $\text{MoO}_3$ ). The solution is acidulated with sulphuric acid (desirably about 1% of the weight of the chromic oxide) to improve its conductivity. The weight of the water in making the bath is desirably from 3 to 10 times that of the chromic oxide. The anode 3 may be formed of some material such as platinum which does not dissolve in the bath during the plating operation, but is desirably formed of molybdenum or chromium-molybdenum alloy which passes into solution during the operation and thereby avoids a depletion of the molybdenum content of the bath. The cathode 4 may be of any shape desired and formed of copper, iron, molybdenum or any conductive material which is desired to plate for any purpose, such for example to protect from oxidation or corrosion by the alloy plating. The plating time depends on the desired thickness of the alloy coating. The proportion of chromic oxide to sulphuric acid is strictly governed by the following formula:

$$\frac{\text{Wt. of } \text{CrO}_3}{\text{Wt. of } \text{H}_2\text{SO}_4 \text{ or its equivalent}} = <100 \text{ or } >50$$

45

The following table gives a summary of some of the work which I have performed in plating metal with chromium-molybdenum alloys.

| Composition of the bath |                  |                                |                  | Anode | Cathode | Current Density, amp./dm. <sup>2</sup> | Time | Temp.  | Thickness of Deposit | Mo in the plate |
|-------------------------|------------------|--------------------------------|------------------|-------|---------|----------------------------------------|------|--------|----------------------|-----------------|
| CrO <sub>3</sub>        | MoO <sub>3</sub> | H <sub>2</sub> SO <sub>4</sub> | H <sub>2</sub> O |       |         |                                        |      |        |                      |                 |
| Grams                   | Grams            | Grams                          | Grams            | Pt.   | Cu.     | Hours                                  | °C.  | Inches | Per Cent             |                 |
| 45                      | 15               | 0.45                           | 300              | Pt.   | Cu.     | 15                                     | 5    | 40     | 0.004                | 4.5             |
| 30                      | 10               | 0.30                           | 200              | Mo    | Cu      | 15                                     | 5    | 40     | 0.003                | 22.4            |
| 60                      | 20               | 0.60                           | 200              | Pt    | Fe      | 25                                     | 5    | 40     | 0.005                | (1)             |
| 20                      | 7                | 0.20                           | 200              | Pt    | Fe      | 15                                     | 5    | room   | 0.004                | (1)             |

<sup>1</sup> Not tested.

From the foregoing disclosure, it will be seen that I have devised a method of plating alloys of chromium and molybdenum from aqueous solutions, said alloys being deposited as dense coherent plate on the cathode of the plating bath. The plating is useful for protecting the plated article from oxidation, chemical corrosion, as well as giving it an attractive finish.

Although a preferred embodiment of my invention has been disclosed, it will be understood that modifications may be made within the spirit and scope of the appended claims.

I claim:

1. The method of electroplating comprising dissolving chromic oxide in from 6 to 7 times its weight of water, dissolving molybdenum trioxide equivalent to about  $\frac{1}{3}$  the weight of chromic oxide in said solution, adding sulphuric acid equivalent to about 1% of the weight of the chromic oxide, heating to a temperature up to 40° C., and passing electric current therethrough, using a base metal cathode and an anode of molybdenum, and continuing the passage of said current for about five hours to form a deposit on the cathode of a molybdenum-chromium alloy containing from 1% to 30% of molybdenum in closely-adherent form.

2. The method of electroplating comprising dissolving chromic oxide in from 6 to 7 times its weight of water, dissolving molybdenum trioxide equivalent to about  $\frac{1}{3}$  the weight of chromic oxide in said solution, adding sulphuric acid equivalent to about 1% of the weight of the chromic oxide,

heating to a temperature up to 40° C., and passing electric current therethrough, using a base metal cathode and an anode of molybdenum, to form a deposit on the cathode of a molybdenum-chromium alloy containing from 1% to 30% of molybdenum in closely-adherent form.

CHUK CHING MA.

#### REFERENCES CITED

The following references are of record in the file of this patent:

#### UNITED STATES PATENTS

| Number    | Name        | Date          |
|-----------|-------------|---------------|
| 1,365,499 | Kelley      | Jan. 11, 1921 |
| 1,581,188 | Fink        | Apr. 20, 1926 |
| 1,717,468 | Schulte     | June 18, 1929 |
| 1,782,092 | Gray et al. | Nov. 18, 1930 |
| 1,795,459 | Westbrook   | Mar. 10, 1931 |
| 1,885,700 | Fink        | Nov. 1, 1932  |
| 1,993,020 | Scott       | Mar. 5, 1935  |
| 2,332,416 | Waltenberg  | Oct. 19, 1943 |
| 2,392,821 | Kreag       | Jan. 15, 1946 |

#### FOREIGN PATENTS

| Number  | Country       | Date           |
|---------|---------------|----------------|
| 240,490 | Great Britain | Sept. 16, 1926 |
| 286,457 | Great Britain | Mar. 8, 1928   |

#### OTHER REFERENCES

J. Am. Chem. Soc., 54, 1932 (3775-6).  
Trans. Electro. Chem. Soc., vol. 70 (1936) pp. 423-429.